

# United States Patent [19]

Iyengar

[11] 3,884,678  
[45] May 20, 1975

[54] FLUXES

[75] Inventor: **Ramachandra K. Iyengar**, Mt.  
Lebanon, Pa.

[73] Assignee: **Jones & Laughlin Steel Corporation**,  
Pittsburgh, Pa.

[22] Filed: **Feb. 4, 1974**

[21] Appl. No.: **439,465**

[52] U.S. Cl. .... **75/52; 75/94**

[51] Int. Cl. .... **C21c 7/00; C22b 9/10**

[58] Field of Search .... **75/52, 53, 94, 5**

[56] References Cited

UNITED STATES PATENTS

3,259,486 7/1966 Kootz..... 75/52

|           |        |               |       |
|-----------|--------|---------------|-------|
| 3,311,465 | 3/1967 | Ban.....      | 75/5  |
| 3,669,618 | 6/1972 | Coppel.....   | 75/94 |
| 3,726,665 | 4/1973 | Minnick.....  | 75/94 |
| 3,793,006 | 2/1974 | Kawawa.....   | 75/94 |
| 3,802,866 | 4/1974 | Rinesch ..... | 75/52 |

Primary Examiner—P. D. Rosenberg  
Attorney, Agent, or Firm—T. A. Zalenski

[57] ABSTRACT

A solid solution of 28 to 32% MnO, 30 to 35% FeO, 25 to 30% CaO and 8 to 12% MgO is advantageously used as a flux, together with external lime, in the refining of steel. As an adjunct, a solid solution of 80% CaO, 15% MnO and 5% FeO is used as a flux without any or with only a minimum of external lime.

6 Claims, No Drawings

## FLUXES

This invention relates generally to fluxes and particularly to fluxes useful in the refining of steel by means of pneumatic steelmaking processes, such as the basic oxygen furnace (BOF) process.

In the refining of molten iron into steel, fluxes are added to the melt primarily for the purpose of reacting with oxidizable impurities in the molten iron to form a slag having the chemical and physical properties necessary for refining the iron to steel in an efficient manner. Sufficient calcium oxide, in the form of lime primarily, is added to the melt to establish a calcium oxide to silicon oxide ratio of at least approximately three to one in order to promote sulfur removal from the molten iron. The silicon oxide is formed, of course, by the oxidation of the silicon in the molten iron. Iron oxide which is both added to the melt and is formed as a result of oxidation of the iron in the melt also acts to flux the lime.

Magnesium oxide is added to create a slag which is essentially saturated in that compound and, thus, minimizes the extraction of magnesium from the refining vessel refractory lining, thereby extending refractory life.

Manganese oxide acts to put lime into solution and to provide the correct fluidity to the slag. This is particularly significant in the BOF process where the proper fluidity is important in minimizing slopping (the ejection of slag from the refining vessel) and the build up of slag on the oxygen lance.

The use of the individual compounds discussed above as slag-forming materials is not new with me. What is new, however, is their introduction into the melt in solid solution. Thus, according to a first embodiment of my invention, a solid solution of 28 to 32% MnO, 30 to 35% FeO, 25 to 30% CaO and 8 to 12% MgO together with external lime are added as the fluxing materials to a pneumatic steel-refining vessel, such as a BOF. In a second embodiment of my invention, an alternate fluxing material consisting of a solid solution of 80% CaO, 15% MnO and 5% FeO is used with little or no external lime.

Since each of the above-mentioned compounds must first go into solution before they can perform their slag functions, I reduce the time of the refining period, i.e., the blowing time in a BOF operation, by adding the compounds in solid solution form. The net effect of adding the compounds in this manner is to create a fluid and reactive slag in a shorter time than is otherwise the case because less thermal and chemical energy is required to develop the proper slag properties.

A better understanding and appreciation of my invention will be had from the following detailed description of the embodiments of the invention as applied to a BOF process.

In the first embodiment of my invention, I take 28 to 32% MnO, 30 to 35% FeO, 25 to 30% CaO and 8 to 12% MgO and form a solid solution of these compounds. By a solid solution, I mean a material where the atomic structure of the manganese, iron, calcium and magnesium is arranged in some coordination with oxygen. The solid solution may be analogized to a steel alloy and is to be clearly distinguished from a mixture of the compounds in which each compound maintains its separate integrity. Preferably, the solid solution consists of 28% MnO, 35% FeO, 25% CaO and 12% MgO.

The solid solution is made by premixing the compounds and thereafter heating the mixture at a temperature and for a time to form the solid solution. The mixture may first be formed into briquettes and then heated or the mixture simply may be sintered. The heating of the mixture to create the solid solution can be effected in various ways. When used in conjunction with the BOF process, the mixture can be heated during the period the BOF vessel is preheated, if preheating is used. Alternatively, the vessel may have sufficient retained heat from a melt which has just been tapped that the mixture need only be injected into the empty vessel and held there for a short time to create the solid solution. Thereafter, the molten iron for the next refining cycle is introduced into the vessel. Additional procedures for heating the mixture to form a solid solution include using waste gas heat from any of the processes producing such heat around a steel plant and external heat sources such as furnaces or kilns.

In a typical BOF steelmaking operation, lime, dolomitic lime and fluorspar are used as the fluxing agents. The lime represents the primary slag-forming ingredient. The dolomitic lime acts primarily to preserve lining life and the fluorspar is added to speed-up the dissolution of the lime.

According to my invention the solid solution of MnO, FeO, CaO and MgO is added to the hot metal in place of the dolomitic lime and fluorspar. However, external lime, that is, lime in addition to that contained in the solid solution is added in conventional quantities less approximately that amount of lime contained in the solid solution. The solid solution flux of my invention reacts rapidly with the silica in the slag to produce a reactive slag in which external lime solution takes place more quickly than through the use of fluorspar; and, of course, in a BOF operation where refining cycle times are measured in terms of minutes, the reduction of the refining cycle even by a few minutes is of significance.

The rapidity with which the solid solution flux of my invention reacts is a result, primarily, of two circumstances: First, because the flux is already in solid solution when added to the molten iron, no energy is required to create a solution of the materials which make up the flux, and the only chemical and thermal energy required is that needed to melt the flux; Second, there is a catalytic effect in the sense that a reactive slag is created at an absolute energy level lower than that which would otherwise be required. In otherwords, if an absolute energy level of  $x$  is required to create a reactive slag in a conventional operation, an absolute energy level of less than  $x$  will produce a reactive slag using the solid solution of my invention.

In the second embodiment of my invention, I provide a flux in which essentially all the lime required is put into solid solution with other fluxing materials and little if any external lime is used. This flux consists of a solid solution of 80% CaO, 15% MnO and 5% FeO. Dolomitic lime can be added externally of the solid solution to extend refractory life.

I claim:

1. A solid solution of flux consisting essentially of 28 to 32% MnO, 30 to 35% FeO, 25 to 30% CaO and 8 to 12% MgO.
2. A solid solution flux encompassed by claim 1 and consisting essentially of 28% MnO, 35% FeO, 25% CaO and 12% MgO.

3. In a pneumatic process for refining iron into steel where lime is added to the iron as a slag-forming ingredient, the improvement comprising also adding a solid solution of a flux consisting essentially of 28 to 32% MnO, 30 to 35% FeO, 25 to 30% CaO and 8 to 12% MgO.

4. The process of claim 3 wherein the solid solution flux consists essentially of 28% MnO, 35% FeO, 25%

CaO and 12% MgO.

5. A solid solution of a flux consisting essentially of approximately 80% CaO, 15% MnO and 5% FeO.

6. In a pneumatic process for refining iron into steel, the improvement comprising adding to the iron a solid solution of a flux consisting essentially of 80% CaO, 15% MnO and 5% FeO.

\* \* \* \* \*

10

15

20

25

30

35

40

45

50

55

60

65